

Oct. 6, 1931.

P. F. LONGNECKER

1,826,622

METHOD OF ROLLING

Filed Oct. 12, 1929

Fig.1.



Fig.2.



Fig.3.



Fig.4.



Fig.5.



Fig.6.



Fig.7.



Fig.8.



Fig.9.



INVENTOR

Paul F. Longnecker

By Byrnes, Stibbing, Pamela & Blakely  
Atty.

## UNITED STATES PATENT OFFICE

PAUL F. LONGNECKER, OF MCKEESPORT, PENNSYLVANIA, ASSIGNOR TO FIRTH-STERLING STEEL COMPANY, OF MCKEESPORT, PENNSYLVANIA, A CORPORATION OF PENNSYLVANIA

## METHOD OF ROLLING

Application filed October 12, 1929. Serial No. 399,257.

This invention relates generally to a method of rolling bodies, such as ingots, blooms or billets, and more particularly to rolling such bodies having deep grooves therein to form sections substantially free from reentrant surfaces.

Many attempts have been made heretofore to provide an ingot of a shape that will decrease or eliminate the objectionable shrinks, pipes and coarse open structure usually found in steel ingots. I have found that if an ingot is cast having deep grooves therein, the amount of shrinks, pipes and coarse open crystalline structure is much less than if the ingot has plain surfaces. I have found that if an ingot in the shape of a cruciform, for example, is cast, it may be rolled so as to make it substantially free from reentrant surfaces. An ingot cast with deep grooves therein has the advantage over other shaped ingots that it is relatively free from the objectionable pipes, shrinks and coarse or open crystalline structure.

This invention relates particularly to a method of rolling ingots having deep grooves to sections substantially free from reentrant surfaces.

In the accompanying drawings which illustrate the present preferred manner of practicing my invention:

Figure 1 is a diagrammatic end elevation of a cruciform ingot; and

Figures 2 to 9, inclusive, illustrate the steps necessary to transform the ingot into a section substantially free from reentrant surfaces.

For illustrative purposes, I have shown a cruciform ingot, but it will be understood that the invention is also applicable to all ingots which are deeply grooved. The cruciform ingot shown in Figure 1 comprises flanges 1, separated by deep grooves 2 and 3. The ingot has two long axes 4, 4 and 4', 4', and two short axes, 5, 5 and 5', 5'. The ingot shown in Figure 1 is fed to reducing rolls 6 (as shown in Figure 2), in order to flatten the edges 7 of the flanges 1. The ingot is fed to the rolls 6 with a short axis 5, 5', extending longitudinally of the rolls. After the ingot has passed through the rolls 6, it is

rotated through substantially 90° and fed through rolls 8 (see Figure 3) which flatten the edges 9 of the ingot. The ingot having its edges flattened is then fed through rolls 10, which reduce the cross section thereof and tend to close the grooves 2. The ingot is then rotated through 90° and is fed to rolls 11 (see Figure 5), which further reduce the cross section thereof and tend to close the grooves 3.

This process of passing the ingot through reducing rolls which tend to close the grooves 2 and 3 and rotating the ingot through 90° between successive passes is carried out until there is danger that the flanges 1 would overlap if the reducing step were carried any further. This reduction of the cross section of the ingot and the closing of the grooves 2 and 3 is preferably carried out by passing the ingot between rolls having substantially plain or smooth surfaces.

When the rolling process has been carried to a point where there is danger that the flanges 1 of the ingot will overlap, it is passed between rolls 12, provided with ribs 13, which contact with the grooves 2 in the ingot and widen them out. The ingot is then rotated through 90° and passed between rolls 14, provided with ribs 15, which contact with and widen out the grooves 3. The ingot is then passed between other sets of rolls which are similar to rolls 14 but each succeeding roll having a rib of decreasing size, and between each pass the ingot is rotated through 90°. Thus from the last mentioned rolls, the ingot passes to rolls 16, is rotated 90°, and then to rolls 17, in which the rib has decreased to such an extent that it is substantially a smooth or plain roll. Thereafter the rolling is continued in any desired manner.

In the method above described, the ingot is subjected to rolling pressure in such direction as to reduce the cross section thereof and to tend to close the grooves 2 and 3. This step is followed by passing the ingot between grooved rolls which reduce the cross section of the ingot and widen out the grooves. The step of closing the grooves is carried out by passing the ingot between smooth rolls and the widening of the grooves is carried out by

- passing the ingot between grooved rolls. In some cases, it may be desirable to first roll the ingot in such a manner as to tend to close the grooves 2 and 3, as illustrated in Figures 2 to 5, then widen the grooves, as illustrated in Figures 6 and 7, then again roll the ingot so as to tend to close the grooves, and then again widen the grooves. The present invention contemplates not only a single rolling step or series of steps tending to close the grooves and a single rolling step or series of steps tending to widen the grooves, but contemplates any number of closing and widening steps or series of steps.
- 15 The above described process enables one to cast an ingot having deep grooves therein which results in an ingot relatively free from shrinks, pipes and coarse crystalline structure, and to thereafter roll the ingot so that it has a cross section substantially free from reentrant surfaces.
- 20 In the claims, the term "edging" is used to define the method of rolling in which the body is rotated through substantially 90° between passes.

I have illustrated and described the present preferred embodiment of my invention, but it will be understood that the invention may be otherwise embodied or practiced within the scope of the following claims.

I claim:

- 35 1. In the method of rolling a deeply grooved body to a section substantially free from reentrant surfaces, the steps comprising applying rolling pressure to the body in direction tending to reduce the cross section thereof and to close the grooves, widening the grooves before laps have formed, and continuing the rolling.
- 40 2. In the method of rolling a deeply grooved body to a section substantially free from reentrant surfaces, the steps comprising applying rolling pressure with substantially smooth rolls to the body in direction tending to reduce the cross section thereof and to close the grooves, widening the grooves before laps have formed, and continuing the rolling.
- 45 3. In the method of rolling a deeply grooved body to a section substantially free from reentrant surfaces, the steps comprising applying rolling pressure to the body in direction tending to reduce the cross section thereof and to close the grooves, engaging the grooves before laps have formed with ribs on the rolls to widen them, and continuing the rolling.
- 50 4. In the method of rolling a deeply grooved body to a section substantially free from reentrant surfaces, the steps comprising applying rolling pressure to the body with substantially smooth rolls in direction tending to reduce the cross section thereof and to close the grooves, engaging the grooves

before laps have formed with ribs on the rolls to widen them, and continuing the rolling.

5. In the method of rolling a deeply grooved body to a section substantially free from reentrant surfaces, the steps comprising feeding the body to a reducing pass with the central plane of a groove in the body extending axially of the rolls forming the pass, and feeding the same to a pass having a ribbed roll effective for widening the groove. 75

6. In the method of rolling a deeply grooved body to a section substantially free from reentrant surfaces, the steps comprising feeding the body to a reducing pass with the central plane of a groove in the body extending axially of the rolls forming the pass, edging the reduced body, and feeding the same to a pass having a ribbed roll effective for widening the groove. 80

7. In the method of rolling a deeply grooved body to a section substantially free from reentrant surfaces, the steps comprising applying rolling pressure to the body in direction tending to reduce the cross section thereof and to close the grooves, and feeding the same through passes having ribbed rolls, the ribs decreasing in size in the successive passes. 85

8. In the method of rolling a cruciform body to a section substantially free from reentrant surfaces, the steps comprising feeding the body through reducing rolls with a short axis of the body extending longitudinally of the rolls, said reduction tending to reduce the grooves between the flanges of the body, and widening the grooves before laps have formed. 95

9. In the method of rolling a cruciform body to a section substantially free from reentrant surfaces, the steps comprising feeding the body through reducing rolls with a short axis of the body extending longitudinally of the rolls, said reduction tending to reduce the grooves between the flanges of the body, edging the reduced body, and widening the grooves before laps have formed. 100

10. In the method of rolling a cruciform body to a section substantially free from reentrant surfaces, the steps comprising feeding the body through reducing rolls with a short axis of the body extending longitudinally of the rolls, rotating the body through substantially 90° and feeding it through reducing rolls with the other short axis of the body extending longitudinally of the rolls, said reductions tending to reduce the grooves between the flanges of the body, and widening the grooves before laps have formed. 110

11. In the method of rolling a cruciform body to a section substantially free from reentrant surfaces, the steps comprising feeding the body through reducing rolls with a short axis of the body extending longitudinally of the rolls, rotating the body through substantially 90° and feeding it through re- 125

ducing rolls with the other short axis of the body extending longitudinally of the rolls, said reductions tending to reduce the grooves between the flanges of the body, and widening the grooves before laps have formed by feeding the body through passes having ribbed rolls which contact with the grooves.

12. In the method of rolling a cruciform body to a section substantially free from re-entrant surfaces, the steps comprising feed-  
10 ing the body between substantially smooth reducing rolls with a short axis of the body extending longitudinally of the rolls, rotat-  
15 ing the body through substantially 90° and feeding it between substantially smooth re-  
ducing rolls with the other short axis of the body extending longitudinally of the rolls, said reductions tending to reduce the grooves between the flanges of the body, and widen-  
20 ing the grooves before laps have formed.

13. In the method of rolling a cruciform body to a section substantially free from re-entrant surfaces, the steps comprising feed-  
25 ing the body between substantially smooth re-  
ducing rolls with a short axis of the body ex-  
tending longitudinally of the rolls, rotating the body through substantially 90° and feed-  
30 ing it to substantially smooth reducing rolls with the other short axis of the body extend-  
35 ing longitudinally of the rolls, said reduc-  
tions tending to reduce the grooves between the flanges of the body, and widening the grooves before laps have formed by feeding the body through passes having ribbed rolls which contact with the grooves.

14. The method of forming an ingot sub-  
stantially free from reentrant surfaces, com-  
prising casting a deeply grooved ingot, ap-  
plying rolling pressure to the ingot in a di-  
40 rection tending to reduce the cross section thereof and to close the grooves, widening the grooves before laps have formed, and continuing the rolling.

15. The method of forming an ingot sub-  
stantially free from reentrant surfaces, com-  
prising casting a cruciform ingot, applying rolling pressure to the ingot in a direction tending to reduce the cross section thereof and to close the grooves, widening the grooves before laps have formed, and continuing the rolling.

In testimony whereof I have hereunto set my hand.

PAUL F. LONGNECKER.